

July 9, 1940.

R. A. HAYWARD

2,207,122

PARCHMENTIZED PAPER

Filed Aug. 25, 1937



BY

FINI INVENTOR.  
Ralph H. Hayward  
Earl & Chappell  
ATTORNEYS

## UNITED STATES PATENT OFFICE

2,207,122

## PARCHMENTIZED PAPER

Ralph A. Hayward, Parchment, Mich., assignor  
to Kalamazoo Vegetable Parchment Company,  
Parchment, Mich.

Application August 25, 1937, Serial No. 160,733

2 Claims. (Cl. 8—119)

This invention relates to improvements in parchmentized paper.

This invention relates to an improved paper and method of making the same, and particularly parchmentized paper designed for wrapping products and for other purposes where substantial strength is desirable.

The main objects of this invention are:

First, to provide an improved parchmentized paper having substantially increased bursting strength, both wet and dry, as compared to standard parchmentized paper of similar stock and weight.

Second, to provide an improved method of manufacturing my improved paper.

Objects relating to details and economies of the invention will appear from the description to follow. The invention is defined and pointed out in the claims.

20 In the accompanying drawing

Fig. 1 is a conventional illustration of parts of an apparatus by which my improved product may be produced, the parchmentizing apparatus other than the washing not being indicated.

25 Fig. 2 is a plan view of a web of paper illustrating the various steps of my method.

In considering the drawing, it will be appreciated that no attempt has been made to show the parts in proportion and that it is not practical to illustrate with great accuracy the creped material or the finished product.

In the shipping and merchandising of various products, parchmentized paper is desirable as, for example, in the crating and shipping of lettuce which is crated wet and frequently with ice enclosed. Also, in packing, the paper is placed in the press with the lettuce with ice and the press actuated to compress the contents into the crate dimensions and this places a severe strain 35 on the paper. Therefore, it is desirable to increase the strength of the paper for this and various other uses. The bursting strength of my paper is very greatly increased over that of paper of similar grades produced by other methods, 40 both as to dry tests and greater increases are found on wet tests, that is, as compared with similar paper produced by other methods.

In the accompanying drawing 1 represents a web of paper to be treated and 2 the washing apparatus for washing the web of paper after it has been subjected to a parchmentizing solution. The apparatus for accomplishing that step is not illustrated as it is well known in the art.

While the paper is wet and preferably while it 55 is still wet from the washing step as illustrated

in Fig. 1, it is passed to a creping apparatus shown conventionally at 3 from which which the creped paper is passed to a drying apparatus. This drying apparatus and particularly the support of the paper during the drying step is of primary 5 importance. When parchment paper is dried by ordinary methods it shrinks very substantially, at least ten inches in a hundred inch width of web. By the usual method of drying parchment paper the paper is held against the flat surface 10 of the drier and instead of the paper shrinking to this full extent there is a tendency for strains to be set up in the paper which reduces the ultimate strength of the sheet.

By my method of this application the parchmentized sheet or web is creped and the creped web is fed to the driers so that it reaches them with the crinkles resulting from the creping still retained therein. The paper is so supported during this drying operation that as the paper 20 shrinks the shrinkage is absorbed by the pockers and issues from the driers with the crinkles of the creping step substantially eliminated. As there has been no strain developed during the 25 drying the strength of the paper is greatly increased in fact, commonly as much as 25% above that of parchmentized paper produced by ordinary methods.

In Fig. 1 of the drawing I illustrate two sections of the driers, that designated by the numeral 4 being provided with the paper felt 5 and that designated by the numeral 6 being provided with a paper carrying felt 7. The crinkled paper indicated at 8 is delivered from the creping rolls to the drier unit 4 which is driven at a certain 30 speed, the speed being controllable by a suitable variable speed drive shown conventionally at 9. The second unit 6 is provided with a variable speed control drive shown conventionally at 10.

The paper is passed from the creping machine 40 directly to the unit 4 which has its individual felt 5. It is passed from the unit 4 to the unit 6 which has its individual felt 7. The unit 4 does not sufficiently heat or dry the paper to result in any substantial shrinkage but as it passes to the unit 6 the paper is subjected to a complete drying 45 which results in shrinkage. However, in view of the paper having been previously creped and being fed through the driers without substantial pull or tension thereon, the shrinkage is compensated for or taken up by the crinkles of the creping step, with the result that by suitably controlling the relative speeds and supporting the paper during the drying the crinkles of the 50 creping step are substantially eliminated, and this 55

without subjecting the fibers to stresses which tend to weaken the sheet or web. If desired the dried sheet may be subjected to a calender stack as indicated at 11 from which it is passed to the 5 winding roll 12.

In Fig. 2 I show a web of paper illustrating the various steps performed thereon, the acid bath step being indicated at 13, the washing at 14, the crinkling at 15 and the drying at 16. I have 10 attempted to illustrate at 16 the gradual elimination of the crinkles by the drying step. The finished paper indicated at 17 is substantially without crinkles resulting from the creping step, although it will be understood that the method 15 may be carried out to such degree as desired.

My parchmentized paper has much greater strength, both wet and dry tests, than paper of the same weight and stock manufactured by commonly practiced methods of making parchmentized paper or any method with which I am familiar. This increased strength, particularly the 20 bursting strength, is easily demonstrated under "Mullen" tests, both dry tests and wet tests.

While I prefer to use kraft paper, any suitable 25 grade of bleached or unbleached or partially bleached stock suitable for parchmentizing may be used. The paper may be manufactured and parchmentized in the usual way, or any preferred

way, and is then subjected to the steps which result in the advantage of greatly increased strength as I have set forth.

Having thus described my invention what I claim as new and desire to secure by Letters Patent is:

1. The method of making substantially smooth parchmentized kraft paper comprising the steps of subjecting a formed sheet or web of kraft paper to a parchmentizing solution, washing, 10 creping the paper while wet, and drying while supported so as to permit shrinkage thereof and the absorption of the shrinkage by the crinkles produced by the creping step and their substantial elimination by such shrinkage. 15

2. The method of producing a substantially smooth parchmentized paper comprising subjecting a form, sheet or web of paper to the steps of parchmentizing, creping, and drying while supported so as to permit shrinkage thereof and the absorption of the shrinkage by the crinkles produced by the creping step and their substantial elimination by such shrinkage, the paper having a "Mullen" test bursting strength substantially higher than parchmentized paper not subjected to such crinkle eliminating, drying and shrinking steps. 20 25

RALPH A. HAYWARD.